

99

Patented Apr. 13, 1926.

1,580,787

from the plate  
then breakT 196  
1/19

## UNITED STATES PATENT OFFICE.

IWAN EMIL LANHOFFER AND OSCAR EDMOND LANHOFFER, OF PARIS, FRANCE, ASSIGNEES TO SIMON J. DANNENBERG, OF NEW YORK, N. Y.

## PROCESS OF PRODUCING HOMOGENEOUS, MOLDABLE POWDERS FROM FIBROUS CEMENTS.

No Drawing.

Application filed March 18, 1925. Serial No. 16,569.

To all whom it may concern:

Be it known that we, IWAN EMIL LANHOFFER, a citizen of the Republic of France, and a resident of Paris, France (post-office address 10<sup>bis</sup> Avenue de la Grande Armee), and OSCAR EDMOND LANHOFFER, citizen of the Republic of France, residing at Paris, France (post-office address 10<sup>bis</sup> Avenue de la Grande Armee), have invented certain new and useful Improvements in a Process of Producing Homogeneous, Moldable Powders from Fibrous Cements, of which the following is a specification.

Whatever the method according to which they are prepared, mortars made of cement and fibrous material hardly offer absolute homogeneity. Hitherto there has been no way to avoid the formation of small bunches of fibres which when such a mortar is spread out in a single layer over a mold plate or other suitable receiving or supporting surface, will of necessity offer points where both resistance and adherence are not the same as with the rest of the mass.

The object of our invention is to provide a process permitting absolute homogeneity to be imparted to such mortars while doing away with the above mentioned defect.

Such process consists in removing from a wet mixture of disintegrated fibrous material and cement constituting the mortar all excess water by compressing said mixture so as to form a block or plate and in subjecting this block or plate to the action of an emery, carborundum or artificial corundum wheel revolving at a high velocity and adapted to reduce it to a moist powder. The process is primarily an improvement on, or development of, the invention disclosed in Patent No. 1,514,666, granted November 11, 1924, to I. E. Lanhoffer, to which reference may be had for a further understanding of some features of the present invention.

We then use this powder either just as it comes from the grinder or after moistening it again when a plastic mortar is desired.

If its peripheral speed is adequate, the wheel itself can be used to produce directly the layer of pulverulent mortar, the latter being dashed by it on the mold plate or other receiving surface.

As will be readily understood, while we consider a grindstone, emery wheel or such like as the best implement to powderize such mortar, we reserve the right to use other means such as cylinders striated like files or rasps, steel bushed, "warped saws," circular saws inclined on their axis of rotation etc., etc., to achieve analogous effects.

Having now particularly ascertained and described the nature of our said invention as well as the manner in which the same is to be performed, we declare that what we claim is:

1. A process of producing homogeneous, moldable powders from fibrous cements, comprising the steps of forming a wet mortar from fibrous material and cement; compressing the mortar into plate or block form to expel all excess water therefrom; and then reducing such plate or block to powder form.

2. A process of producing homogeneous, moldable powders from fibrous cements, comprising the steps of forming a wet mortar from fibrous material and cement; compressing the mortar into plate or block form to expel all excess water therefrom; and then subjecting the plate or block to the action of a rapidly-rotating grinding element to reduce it to the form of a moist powder.

In testimony whereof we affix our signatures.

IWAN EMIL LANHOFFER.  
OSCAR EDMOND LANHOFFER.